

# UNITED STATES PATENT OFFICE.

JOHN M. CALLOW, OF SALT LAKE CITY, UTAH, ASSIGNOR TO METALS RECOVERY COMPANY, OF AUGUSTA, MAINE. A CORPORATION OF MAINE.

## PROCESS OF CONCENTRATING ORES.

1,269,157.

Specification of Letters Patent. Patented June 11, 1918.

No Drawing.

Application filed November 2, 1916. Serial No. 129,154.

To all whom it may concern:

Be it known that I, JOHN M. CALLOW, a subject of the King of Great Britain, residing at Salt Lake City, in the county of 5 Salt Lake and State of Utah, have invented certain new and useful Improvements in Processes of Concentrating Ores, of which the following is a specification.

This invention relates to a new and useful process of concentrating ores, and it has for its essential object the separation of an ore relatively high in certain values, from other products relatively high in other values.

15 With the above and other objects in view, my invention consists of the process substantially as I will hereinafter describe and claim.

In carrying out my invention I take advantage of the well-known action of frothing and floating oils, when used with any of the suitable and well-known flotation apparatus, in connection with a certain class of chemicals, commonly known as salt-cake 20 and niter-cake, which are by-products derived from powder and other chemical manufacturing plants.

My process is applicable to and is intended to cover the use of sodium-hydrogen-sulfate or sodium-acid-sulfate commonly known as salt-cake or niter-cake in any froth-flotation apparatus with crushed crude copper, lead, zinc, iron, etc., ores, slimes, tailings, middlings or concentrates 25 where the selective action of one metallic constituent of the ore mass is preferential to the others. The action of the sodium-hydrogen-sulfate or sodium-acid-sulfate in the ore mass is to immunize against flotation one or more of the mineral components of a mixture of mineral particles each normally susceptible to flotation and, therefore, my process is based upon the fact that when an ore, slime, concentrate, etc., ground 40 to a fineness necessary to separate the various constituents, is treated with sodium-hydrogen-sulfate in quantity sufficient to immunize against flotation certain of the mineral components normally susceptible to flotation, or is likewise treated with salt cake, or niter cake, and an acid, preferably sulfuric acid, and a frothing agent added, and the whole placed in a flotation apparatus, there will be a preferential action of

one or more of the valuable constituents of 55 the ore over the others. As illustrative of one example of my process, I have taken a lead, zinc, iron sulfid, assaying 14% lead, 18% iron, and 16½% zinc, and ground this mixture with an appropriate frothing agent 60 or agents to a fineness sufficient to liberate the various metals. After such grinding, I added the niter-cake, in the proportion or ratio of about 100 pounds per ton of ore-feed, with its usual liquid content. Thus 65 pulp was placed in an appropriate froth-producing apparatus or flotation cell and was thoroughly mixed and, approximately, 2 pounds of commercial sulfuric acid was added and the pulp subjected to the usual 70 step of flotation. As a result of this operation, the froth concentrates assayed about 5% lead, 45% zinc, 7% iron, and 3% of insoluble. The tailings were treated upon appropriate concentrating tables to remove as 75 associated silica, and were found to assay about 30% lead, 6% zinc, 25% iron, and 1% of insolubles. The final tailings assayed approximately, 3% lead and 3% zinc.

I have also found that the crude ore can 80 all be floated free from gangue and then treated as above described so as to give two grades of concentrates.

The foregoing process is applicable to 85 oxides and carbonates or ores which can be film or sulfidized.

It will be understood that the exact proportion of the salt-cake or niter-cake or salt-cake or niter-cake and an acid heretofore described in the working of my process 90 is not absolutely necessary, and hence I desire to state that my process comprehends and includes the use of salt-cake or niter-cake or salt-cake or niter-cake and an acid in other and different proportions from 95 those heretofore given, and that the proportion will be determined according to the particular characteristics of the individual ore to be treated.

From the foregoing it will be understood 100 that I have produced a process of concentrating ores by subjecting the ore to the action of salt cake or niter cake, or salt cake or niter cake and an acid and then treating the pulp by flotation separation whereby I 105 obtain products, some of which are relatively high in certain values and others are relatively high in other values.

Having thus described my invention what I claim as new and desire to secure by Letters Patent is:—

1. The process herein described of concentrating metalliferous ores, which consists in subjecting a pulp of powdered ore and water to the action of sodium-hydrogen-sulfate in quantity sufficient to immunize against flotation certain of the mineral components normally susceptible to flotation, and then subjecting the mass to flotation separation whereby products are obtained relatively high in certain values and other products are obtained relatively high in other values.
2. The process herein described of concentrating metalliferous ores which consists in subjecting a pulp of powdered ore and water to digestion in a solution of sodium-hydrogen-sulfate in quantity sufficient to immunize against flotation certain of the mineral components normally susceptible to flotation, and then subjecting the mass to flotation separation to obtain products relatively high in certain values and other products relatively high in other values.
3. The process herein described of con-

centrating metalliferous ores which consists in reducing the ore in the presence of an appropriate frothing agent to a fineness sufficient to liberate the various metallic constituents of the ore; adding to the ground mass sodium-hydrogen-sulfate in quantity, sufficient to immunize against flotation certain of the mineral components normally susceptible to flotation, and then treating the mass to flotation separation.

4. The process herein described of concentrating metalliferous ores which consists in reducing the ore in the presence of an appropriate frothing agent to a fineness sufficient to liberate the various metallic constituents of the ore, adding to the ground mass sodium-hydrogen-sulfate in quantity sufficient to immunize against flotation certain of the mineral components normally susceptible to flotation and an acid to thereby secure preferential selective action of one metallic constituent of the ore mass to the others, and then treating the mass to flotation separation.

In testimony whereof I affix my signature.

JOHN M. CALLOW.